

## UNITED STATES PATENT OFFICE

2,136,341

## FLOTATION OF CULM

Norman Hedley, Westfield, N. J., assignor to  
 American Cyanamid Company, New York,  
 N. Y., a corporation of Maine

No Drawing. Application September 1, 1936,  
 Serial No. 98,975

4 Claims. (Cl. 209—166)

This invention relates to the flotation of slush culm and other refuse coal. In a more specific modification, the invention is especially concerned with the recovery of low ash coal from anthracite slush culm or other anthracite refuse.

The problem of coal refuse, both bituminous and anthracite, has long been a serious one in the industry. The refuse coal is mainly contaminated with high ash material and is not useable as such. As a result, serious losses of good coal in fine sizes are suffered by the industry, and they have to incur considerable expense in disposing of the slush culm which is usually pumped into large culm banks. Many mines do not have sufficient fairly level ground for culm banks and when the banks are placed on too great a slope, rain washes the coal into the rivers and a serious nuisance frequently arises. Slush culm banks, particularly bituminous coal, also tend to ignite and burn for years with serious annoyance from smoke and fumes. The losses represented by the good coal in the culm or other refuse are, of course, much more serious in the anthracite industry than in the bituminous industry, because the unit value of anthracite coal is higher than bituminous and the character of the anthracite coal results in greater degradation in the breaker and hence larger proportions of the slush culm.

Flotation of coal refuse has been proposed and has been used fairly extensively in Europe primarily with bituminous and semi-bituminous coal. In the United States, owing to the very low price of bituminous coal in the last few years, coal flotation has been employed sporadically only by a few companies. Efforts to float good coal out of anthracite refuse have proven to be complete failures in the past and even with bituminous coal the operations have not been successful in the United States, despite the fact that bituminous coal represents a somewhat easier flotation problem.

When refuse coal is floated, such as anthracite slush culm, and in the following more specific discussion of the invention the description will be based on the purification of anthracite slush culm although it should be understood that the features are also applicable to bituminous coal, the culm contains a mixture of materials varying both in size and in composition. That is to say, there is a certain amount of coal, for example about 60% in representative anthracite culms, which is very low in ash, containing less than 10% of ash and approaching the actual inherent coal ash for coal from that particular area. This good coal occurs in a wide range of sizes running from  $\frac{3}{4}$ " down to very fine particles less than 100 mesh (Tyler Standard Series). The accompanying 40% of higher ash material, of course, grades from material with only slightly higher ash than

the good coal, down to material which is mostly ash with only little coal. This high ash material also occurs in practically as wide a range of size as the good coal.

The flotation of coal, using standard flotation reagents which are for the most part hydrocarbons such as kerosene accompanied, if necessary, by suitable frothers, is based on wettability of the coal by the oil and the coal therefore tends to attach itself to the froth bubbles and appears in the concentrate. Since, however, the material present in the culm grades all the way from pure coal (having only inherent ash) to a slaty gangue impregnated with small amounts of coal, it is difficult and has hitherto been impossible to obtain a sharp flotation separation with good recovery such as is commonly found in the flotation of sulfide minerals and free gold because the good coal is not entirely liberated from the gangue. The problem might be considered as one in which it was necessary to float a concentrate of mineral values away from a partly mineralized gangue. Due to the fact that the coal to be recovered forms a large proportion of the feed, usually somewhat over half, a very large bulk of concentrate is produced which puts a heavy load on the flotation machines and renders the problem even more difficult.

The goal of a flotation cleaned coal from anthracite culm is less than 10% ash. It has been proposed to float slush culm by grinding down to a uniform fine size. These proposals are without economic value as the grinding plant is as large as the flotation plant and the result of grinding reduces the value of the clean coal obtained. Previous attempts to clean anthracite slush culm followed the general flotation procedure which has been used with slight success on bituminous coal; that is to say, the culm with or without grinding, is floated in a string of flotation machines using cleaner machines for cleaning the concentrate. There is no difficulty in obtaining a concentrate which contains a large portion of the good coal, say from 80% up, but such a concentrate is not low in ash and cannot be economically cleaned. Attempts to improve the grade of the coal concentrate by reducing the amount of reagents used were also unsuccessful. It was possible to obtain a concentrate of the desired ash content but only at the expense of very serious losses in recovery. All attempts to vary flotation procedure failed to produce both good recovery and a low ash concentrate.

The present invention is based on the discovery that it is possible to float a full size range of refuse coal such as anthracite slush culm, with a very small amount of reagents so that a concentrate is obtained containing the finer particles of low ash coal and substantially uncontaminated by any considerable portions of

high ash material. This concentrate, which is of high grade ash, represents only a relatively small recovery as the coarser coal of low ash content is not floated. The tailings contain 5 coarse low ash coal and also a large amount of high ash material. The tailings are sized or classified preferably by screening and the fine material which consists almost exclusively of fine high ash material, is rejected. The coarser 10 material, while it contains all of the coarse low ash coal, is still contaminated with a certain amount of coarse high ash material, and therefore screening of the tailings will not recover the coarse coal in the form of a sufficiently low 15 ash material. However, the oversize from the classification of the tailings can then be floated under conditions which will result in the flotation of coarse low ash coal particles and difficulties will not be encountered because the high 20 ash material is all likewise coarse and therefore does not float off into the concentrate and the problem of contamination with high ash material is solved.

The present invention not only results in obtaining a better recovery of low ash material, 25 but also results in an increased capacity of flotation equipment. The consumption of collector which is usually kerosene or a similar hydrocarbon, is also decreased.

It is an advantage of the present invention 30 that the standard reagents can be used. However, it has been found that a frother consisting of paraffin alcohols of 7 to 10 carbon atoms stabilized with a hydrocarbon gives better 35 results and in a more specific aspect the invention includes this feature.

While the invention may be used with any type 40 of flotation machine, best results are obtained with mechanical machines. Some mechanical machines tend to break down and degrade the coal and therefore transform a considerable amount of the coarser material into less valuable fine material. I have found that best results are obtained in machines of the Fagergren type, 45 producing a minimum of degradation and which are well suited for floating the wide range of sizes which is necessary in carrying out the present invention.

The process of the invention is very flexible 50 and is well adapted to handle refuse coal of different types to produce products for various markets. Thus, for example, in many cases there is a good market at a higher price for coarser coal sizes and it is desirable to keep 55 the fine rougher concentrate separate from the floated coarse portion of the tailings. In other cases, for example where the clean coal is to be pulverized, it may be desirable to mix the two final products together.

Where the ash requirements are not unduly 60 severe, the rougher concentrate may remain uncleaned but where the minimum ash is required, it is desirable to clean the rougher concentrate as such a cleaning operation will greatly reduce 65 the ash without material loss in good coal. Of coarse, the additional cleaning operation of the rougher concentrate necessitates additional flotation equipment and slightly increases the amount of reagents. The particular compromise 70 best suited for any given condition is largely determined by economic considerations and it is an advantage of the present invention that it is flexible and that the best and most profitable compromise can be chosen.

The invention will be described in greater de-

tail in conjunction with the cleaning of anthracite slush culm from the bank or current production of the Philadelphia & Reading Coal & Iron Company. It should be understood that the exact details of flotation type, reagent consumption, and the like, will vary somewhat with different culm and with different coals, and the invention is therefore in no sense limited to the precise details of the specific examples.

#### Example 1

Slush culm from the Locust-Summit Breaker of the Philadelphia & Reading Coal & Iron Company was floated in standard Fagergren flotation machines with .276 lb. per ton of a frother 15 consisting of a mixture of paraffin alcohols of 7 to 10 carbon atoms and stabilized with a hydrocarbon, and which is described in the patent of Christmann and Jayne No. 2,065,053 issued December 22, 1936, without any hydrocarbon collector. A concentrate was obtained which contained fine coal only, then the tails were classified in the presence of 0.5 lb. per ton of sodium silicate and after rejection of the finer material 5 lbs. per ton of kerosene were added to the residual pump at about 50% solids and the pulp then diluted to 20% solids and floated in a second set of flotation machines.

The original culm had an ash content of 25-26%, and the results obtained by the treatment are summarized in the following table:

| Product             | Weight, percent | Ash, percent | Cumulative      |              | 35 |
|---------------------|-----------------|--------------|-----------------|--------------|----|
|                     |                 |              | Weight, percent | Ash, percent |    |
| Conc. 1.....        | 26.56           | 12.1         | 26.56           | 12.1         |    |
| Conc. 2.....        | 44.14           | 11.0         | 70.70           | 11.4         |    |
| Tail.....           | 16.55           | 56.0         | 87.25           | 19.9         |    |
| Rejected fines..... | 12.75           | 62.2         | 100.00          | 25.3         | 40 |

#### Example 2

High ash slush culm from the Locust-Summit Breaker of the Philadelphia & Reading Coal & Iron Company having approximately 40% ash, 45 was floated at 21% solids in standard Fagergren flotation machines with .0322 lb. per ton of the frother described in Example 1. A rougher concentrate is obtained which contains the fine low ash coal. The remaining pulp is then screened at 28 mesh and .092 lb. per ton of frother and 4 lbs. per ton of kerosene added to the +28 mesh material. This coarse material is floated to give a second rougher concentrate, and both rougher concentrates are cleaned using .092 lb. per ton of additional frother in each case. The results obtained are shown in the following table:

| Product                              | Individual   |              | Cumulative   |              | 60 |
|--------------------------------------|--------------|--------------|--------------|--------------|----|
|                                      | Wt., percent | Ash, percent | Wt., percent | Ash, percent |    |
| Cl. conc. 1.....                     | 30.34        | 10.0         | 30.34        | 10.0         |    |
| Cl. tail 1.....                      | 2.88         | 70.2         | 33.22        | 15.2         |    |
| Cl. conc. 2.....                     | 28.47        | 15.3         | 61.69        | 15.25        |    |
| Cl. tail 2.....                      | 1.01         | 62.0         | 62.70        | 16.0         |    |
| R. tail.....                         | 16.10        | 83.8         | 78.80        | 29.9         |    |
| -28 mesh reject.....                 | 21.20        | 74.0         | 100.00       | 39.2         |    |
| Composite of cl. concs. 1 and 2..... |              |              | 58.81        | 12.57        | 65 |
| Composite of waste products.....     |              |              | 41.19        | 77.2         | 70 |

In the claims the term "coal of froth flotation size" is intended to cover coal of a size passing through 10 mesh screens and has no other mean-

ing. This represents about the coarsest coal which can be floated by a froth flotation process.

What I claim is:

- 5 1. A method of cleaning refuse coal which comprises subjecting the refuse coal of froth flotation size to a froth flotation process with an amount of reagent insufficient to float fine high ash particles whereby a concentrate is produced containing a major portion of fine low ash coal particles, classifying the flotation tailings, rejecting the fine sizes and subjecting the coarse sizes to froth flotation with an amount of flotation reagent sufficient to float coarse low ash particles.
- 10 10 2. A method of cleaning anthracite slush culm which comprises subjecting the anthracite slush

culm of froth flotation size to a froth flotation process with an amount of reagent insufficient to float fine high ash particles whereby a concentrate is produced containing a major portion of fine low-ash coal particles, classifying the flotation tailings, rejecting the fine sizes and subjecting the coarse sizes to froth flotation with an amount of flotation reagent sufficient to float coarse low ash particles. 5

3. A method according to claim 2 in which the classification is effected by screening. 10

4. A method according to claim 2 in which the tailing is sized on a screen at approximately 28 mesh.

NORMAN HEDLEY. 15